

Oct. 5, 1948.

B. H. CARROLL ET AL  
PHOTOGRAPHIC SILVER HALIDE EMULSION SUPERSENSITIZED  
WITH A C-ACETOXY QUINOLINE BASE  
Filed April 20, 1946

2,450,748



A = 3,3'-diethyl-9-methylselenacarbocyanine bromide

B = 3,3'-diethyl-9-methylselenacarbocyanine bromide  
plus 6-acetoxyquinoline

Burt H. Carroll  
John Spence  
INVENTORS

BY *N. M. Perrins*  
*Daniel J. Mayne*  
ATTORNEYS

## UNITED STATES PATENT OFFICE

2,450,748

PHOTOGRAPHIC SILVER HALIDE EMULSION  
SUPERSENSITIZED WITH A C-ACYLOXY  
QUINOLINE BASEBurt H. Carroll and John Spence, Rochester,  
N. Y., assignors to Eastman Kodak Company,  
Rochester, N. Y., a corporation of New Jersey

Application April 20, 1946, Serial No. 663,762

9 Claims. (Cl. 95—7)

1

This invention relates to sensitized photographic emulsions and to a process for preparing the same. This application is a continuation-in-part of our copending application Serial No. 466,796, filed November 24, 1942 (now United States Patent 2,398,778, dated April 23, 1946).

It is known that the distribution of spectral sensitivity of certain spectrally sensitized emulsions can be altered and an increase of sensitivity obtained in some spectral region by incorporating certain additional sensitizing dyes in the spectrally sensitized emulsions (see United States Patent 2,158,882, dated May 16, 1939, and 2,159,565, dated May 23, 1939). The effect thus produced has come to be known as supersensitization. Supersensitization of certain spectrally sensitized emulsions can also be effected by incorporating certain substantially colorless heterocyclic bases, viz. those containing an amino group, in the spectrally sensitized emulsions. (See United States Patent 2,177,635, dated October 31, 1939.) Supersensitization differs from hypersensitization which involves treatment of finished films or plates, an operation which normally reduces the pAg and increases the pH of the emulsion, with consequent decreased stability.

We have now found a new method for supersensitizing spectrally sensitized emulsions, which not only does not reduce the stability of the emulsions, but is especially valuable as a means of giving good panchromatic sensitized emulsions of high speed and good color balance.

It is, accordingly, an object of our invention to provide new supersensitized photographic emulsions. A further object is to provide a process for preparing such emulsions. Other objects will become apparent hereinafter.

In accordance with the invention, a photographic silver halide emulsion other than a chloride emulsion, e. g. silver chlorobromide (which may contain small amounts of silver iodide), silver bromide or silver bromoiodide emulsions, spectrally sensitized with a (at least one) cyanine dye is supersensitized by incorporating in the emulsion a (at least one) quinoline base containing an (at least one) acyloxy (acyloxy) group attached to a (at least one) carbon atom of the quinoline base. Our invention is directed principally to emulsions of such grain size that the

2

emulsions give a substantially neutral-toned image in Eastman Kodak Company's "D-76" developer, and should not be confused with prior proposals to obtain blue-black tones in fine-grain emulsions by means of heterocyclic nitrogen bases. Moreover, our invention involves incorporation of the quinoline bases in the emulsion before exposure of the emulsion and should not be confused with proposals to develop with color-forming developers silver salt images, in the presence of certain heterocyclic nitrogen bases which contain a reactive methyl group.

The quinoline bases employed in practicing our invention are quinoline bases containing an acyloxy group attached to a carbon atom of the quinoline base. Advantageously the acyloxy group is an acetoxy group or a benzoxy group. Examples of the acyloxyquinolines include 6-acetoxyquinoline, 2-acetoxyquinoline, 6-benzoxyquinoline, etc.

The majority of cyanine dyes which are supersensitized by the quinoline bases are characterized by the fact that the dyes produce two types of sensitization depending upon conditions. Such 25 different types of sensitization are described by Leermakers, Carroll and Staud, J. Chem. Physics 5, 878 (1937) and by Schwarz, Sci. et Ind. Phot. 10, 233 (1939). When a cyanine dye of this type is used as a sensitizer in low concentration, it exhibits a sensitizing maximum displaced about 20 30 to 50  $\mu$  toward the red from the absorption maximum in ethyl alcohol solution. On increasing the concentration of the dye, or upon digesting the emulsion containing the dye in the lower concentration, or both, a second maximum of sensitization develops at longer wavelengths, which may be accompanied by an increase in total optical sensitization. In some cases, a decrease in sensitivity at the first maximum can be detected. These phenomena are consistent with the hypothesis of two states of the sensitizing dye in an equilibrium which is controlled by concentration. The quinoline bases favor the formation of a second maximum which occasionally is appreciably displaced from the normal second maximum. The increase in sensitivity apparently corresponds to increased conversion of the dye to the state corresponding to the second maximum of sensitization. In some cases, the effect

appears to correspond to a more complete conversion than has ever been obtained without a supersensitizer, and in any case the long wavelength sensitivity is better than can be obtained from the same concentration of dye without the quinoline base.

The following are exemplary of the cyanine dyes which are supersensitized in accordance with our invention:

3,1'-diethyl-6'-methoxy-2'-cyanine iodide  
 3,3'-diethyl-9-methylthiacarbocyanine bromide  
 9-ethyl-3,3'-dimethylthiacarbocyanine bromide  
 5'-chloro-3,3',9-triethylthiacarbocyanine iodide  
 5,5'-dichloro-3,3',9-triethylthiacarbocyanine iodide  
 3,3'-diethyl-9-methyl-4,5,4',5'-dibenzothiacarbocyanine bromide  
 3,3'-diethyl-9-methylselenathiacarbocyanine bromide  
 5'-chloro-3,3'-diethyl-9-methylselenathiacarbocyanine iodide  
 3,3'-diethyl-9-methylselenacarbocyanine bromide  
 1'-ethyl-3,6'-dimethyl-4-phenylthiazolo-2'-cyanine bromide  
 3,1'-diethyl-6'-methoxythia-2'-cyanine bromide  
 1,1'-diethyl-2,2'-cyanine bromide  
 1,1'-diethyl-2,2'-carbocyanine bromide  
 9-ethyl-3,1'-dimethylthia-2'-carbocyanine iodide  
 3,3'-diethyl-9-methyl-5-phenoloxathiacarbocyanine iodide  
 3,3'-diethyloxatricarbocyanine iodide

The sensitizing dyes can be employed in any desired concentration. Ordinarily from 10 to 30 mg. of dye per liter of emulsion will suffice to produce the optimum sensitizing effect. The methods of incorporating sensitizing dyes in emulsions are well known to those skilled in the art. Ordinarily it is preferable to dissolve the dye in a water-miscible solvent, such as methanol or ethanol, before incorporating in the emulsion. One or more sensitizing dyes can be employed.

The amount of quinoline base employed is not critical. Usually the full supersensitizing effect is developed at a concentration of 0.10 to 1.5 grams per liter of emulsion. At these concentrations practically none of the quinoline bases has an appreciable effect on the pH of the emulsion. The quinoline bases can be added to the emulsions with, before or after the sensitizing dye or dyes. More than one quinoline base can be employed. The quinoline bases are preferably, but not necessarily, diluted with a water-miscible solvent, such as methanol, before incorporation in the emulsions. The sensitizing dye or dyes and the quinoline base or bases can be added to the emulsions at any convenient stage of their preparation, but preferably to the washed, finished emulsions before coating.

The following example will serve to illustrate further the results obtained in accordance with our invention.

#### Example

A fast negative gelatino-silver-bromiodide developing-out emulsion was sensitized with 3,3'-diethyl-9-methylselenacarbocyanine bromide (20 mg. per liter of emulsion) and to a portion of the spectrally sensitized emulsion was added 6-acetoxyquinoline. A portion of the spectrally sensitized emulsion without the 6-acetoxyquinoline and a portion containing it were exposed through red (Wratten No. 25) and minus blue

(Wratten No. 12) filters. The results are tabulated below:

| 5    | 6-acetoxyquinoline (cc. per liter of emulsion) | Red   |       | Minus Blue |       |
|------|------------------------------------------------|-------|-------|------------|-------|
|      |                                                | Speed | Gamma | Speed      | Gamma |
|      |                                                |       |       | 10         | 10    |
| none |                                                | 119   | 1.47  | 435        | 1.59  |
| 0.25 |                                                | 187   | 1.89  | 555        | 1.87  |
| 0.50 |                                                | 260   | 1.74  | 550        | 1.92  |

Similarly 6-benzoxyquinoline and other quinoline bases containing an acyloxy group supersensitize the emulsions spectrally sensitized with cyanine dyes. Some of the quinoline bases while effecting an increase of sensitivity (speed) in some spectral region, cause a decrease in others, and must be employed with that fact in mind.

The accompanying drawing illustrates graphically the supersensitizing effect obtained with one of our new combinations in a gelatino-silver-bromiodide emulsion. The figure is a diagrammatic reproduction of two spectrograms. Curve A represents the sensitivity of the emulsion sensitized with 3,3'-diethyl-9-methylselenacarbocyanine bromide in a concentration of 20 mg. per liter of emulsion. Curve B represents the sensitivity of the same emulsion sensitized with 3,3'-diethyl-9-methylselenacarbocyanine bromide in a concentration of 20 mg. per liter of emulsion, 6-acetoxyquinoline having also been added to the emulsion in a concentration of 0.25 cc. per liter of emulsion. The supersensitizing or synergistic effect of the combination is apparent. 6-Acetoxyquinoline, alone, imparts no additional spectral sensitivity to the emulsion.

Our invention is primarily directed to the customarily employed gelatino-silver-halide developing-out emulsions, such as gelatino-silver-chlorobromide, gelatino-silver-bromide and gelatino-silver-bromiodide developing-out emulsions, especially emulsions for development to black-and-white images by means of non-color-forming developers, e. g. hydroquinone-N-methyl-p-aminophenol developers.

Emulsions prepared in accordance with our invention can be coated in the usual manner upon any desired support, such as cellulose nitrate support, cellulose acetate support, polyvinyl acetal resin support, metal support, glass support or paper support.

What we claim as our invention and desire to be secured by Letters Patent of the United States is:

1. A photographic silver halide emulsion selected from the group consisting of silver chlorobromide, silver bromide and silver bromiodide emulsions spectrally sensitized with a sensitizing cyanine dye containing, as a supersensitizer, a quinoline base containing an acyloxy group attached to a carbon atom of the quinoline base.
2. A photographic silver halide developing-out emulsion selected from the group consisting of silver chlorobromide, silver bromide and silver bromiodide developing-out emulsions spectrally sensitized with a sensitizing cyanine dye containing, as a supersensitizer, a quinoline base containing an acyloxy group attached to a carbon atom of the quinoline base.
3. A photographic gelatino-silver-halide developing-out emulsion selected from the group consisting of gelatino-silver-chlorobromide, gelatino-silver-bromide and gelatino-silver-bromiodide developing-out emulsions spectrally sensitized with a sensitizing cyanine dye containing,

as a supersensitizer, a quinoline base containing an acyloxy group attached to a carbon atom of the quinoline base.

4. A photographic gelatino-silver-bromiodide developing-out emulsion spectrally sensitized with a sensitizing cyanine dye and containing, as a supersensitizer, a quinoline base containing an acyloxy group attached to a carbon atom of the quinoline base.

5. A photographic gelatino-silver-halide developing-out emulsion selected from the group consisting of gelatino-silver-chlorobromide, gelatino-silver-bromide and gelatino-silver-bromiodide developing-out emulsions spectrally sensitized with a cyanine dye which produces a maximum of spectral sensitivity in the emulsion at one concentration and at a higher concentration, or upon digestion of the emulsion at the lower concentration, produces a second maximum of spectral sensitivity at a wavelength longer than that of the first maximum, said emulsion containing as a supersensitizer, a quinoline base containing an acyloxy group attached to a carbon atom of the quinoline base.

6. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion at the lower concentration, produces a second maximum of spectral sensitivity at a wavelength longer than that of the first maximum, said emulsion containing as a supersensitizer, a quinoline base containing an acetoxy group attached to a carbon atom of the quinoline base.

7. A photographic gelatino-silver-bromiodide developing-out emulsion spectrally sensitized with a cyanine dye which produces a maximum of

6  
spectral sensitivity in the emulsion at one concentration and at a higher concentration, or upon digestion of the emulsion at the lower concentration, produces a second maximum of spectral sensitivity at a wavelength longer than that of the first maximum, said emulsion containing, as a supersensitizer, 6-acetoxyquinoline.

8. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion at the lower concentration, produces a second maximum of spectral sensitivity at a wavelength longer than that of the first maximum, said emulsion containing, as a supersensitizer, a quinoline base containing a benzoxy group attached to a carbon atom of the quinoline base.

9. A photographic gelatino-silver-bromiodide developing-out emulsion spectrally sensitized with a cyanine dye which produces a maximum of spectral sensitivity in the emulsion at one concentration and at a higher concentration, or upon digestion of the emulsion at the lower concentration, produces a second maximum of spectral sensitivity at a wavelength longer than that of the first maximum, said emulsion containing, as a supersensitizer, 6-benzoxyquinoline.

BURT H. CARROLL.  
JOHN SPENCE.

#### REFERENCES CITED

The following references are of record in the  
35 file of this patent:

#### UNITED STATES PATENTS

| Number    | Name | Date         |
|-----------|------|--------------|
| 2,158,882 | Mees | May 16, 1939 |